# EUROPEAN PATENT SPECIFICATION

(11) **EP 0 038 136 B1**
(45) Date of publication and mention of the grant of the patent: **05.06.1985**
(21) Application number: 81301359.6
(22) Date of filing: 27.03.1981
(51) Int. Cl.: D21H 5/20

(54) **Fibrous materials**
Fasermaterialien
Matières fibreuses

(30) Priority: 16.04.1980 GB 8012488; 29.07.1980 GB 8024696
(43) Date of publication of application: 21.10.1981
(73) Proprietor: IMPERIAL CHEMICAL INDUSTRIES PLC, London SW1P 3JF (GB)
(72) Inventor: Ragg, Pudens Leonard, Stockton-on-Tees Cleveland (GB); Smeeton, Roy, Stockton-on-Tees Cleveland (GB); Martin, Graham Ernest, Middlesbrough Cleveland (GB)
(74) Representative: Gratwick, Christopher

## Description

This invention relates to fibrous materials and in particular to sheet-like articles containing amino-formaldehyde resin fibres.

Amino-formaldehyde resin fibres are useful as the fibrous constituents in sheet like articles such as paper where they are generally used in admixture with cellulosic fibres.

Papers made wholly from amino-formaldehyde resin fibres tend to have little or no strength because generally the fibres exhibit little or no self adhesion. When blended with cellulosic fibres, the latter donate strength to the paper but in many cases it would be desirable to improve the strength still further.

One way of improving the strength is to employ partially cured (degree of cure 50-90%) amino-formaldehyde resin fibres. Thus in EP-A-14026, paper is made from partially cured amino-formaldehyde resin fibres made by employing only mild curing conditions, i.e. weak curing catalysts, low curing temperatures and/or short curing times. Partially cured amino-formaldehyde resin fibres can also be made as described in US Patent 4172057 by conducting the reaction of the amino compound with the formaldehyde in the presence of certain carbohydrates.

The degree of cure of amino-formaldehyde resin fibres is measured by digesting an accurately weighed sample (about 5 g) of the dry fibre in 200 ml of water for 2 hours at 50°C. The undissolved fibre is recovered by filtration, dried at 100°C in air for 2 hours, and then reweighed. The degree of cure is the ratio between the weight of the recovered fibre and the original weight of fibre, and is expressed herein as a percentage.

While amino-formaldehyde resin fibres that have only been partially cured may exhibit some self adhesion and so be used as the sole fibrous component of paper, they suffer from the disadvantages that some of the fibre may be lost during the conventional wet-laid paper production process because of the partial water solubility of the partially cured resin and also that free formaldehyde may be evolved during the paper making process thus constituting a health hazard.

It has now found that, under certain conditions, articles, e.g. paper, of improved strength, containing amino-formaldehyde resin fibres having a higher degree of cure can be made.

In the present invention, the processing conditions are such as to cause welding of the amino-formaldehyde resin fibres to each other and/or to other fibrous materials present at at least some of the points where the fibres contact one another. Such welding is referred to herein as inter-fibre bonding. Inter-fibre bonding can be observed using a microscope: thus if a sample of the article, e.g. paper, is observed using a magnification of x 100 or greater, welds between at least some of the fibres can be seen. It will be appreciated that it is not necessary, in order to obtain useful improvements in strength, that every fibre should be welded to another fibre. However the degree of inter-fibre bonding should preferably be such that less than 50% by weight of the amino-formaldehyde resin fibres can be removed from the sample as individual fibres without any fibres adhering thereto when the sample is probed with a fine probe. In the present invention inter-fibre bonding is achieved with highly cured amino-formaldehyde resin fibres, i.e. those having a degree of cure above 93%, by heating the sheet material in the presence of water under specified conditions.

It has been proposed in FR-A-2373617 to dry paper made from certain amino-formaldehyde resin fibres by heating at above 60°C and to improve the cohesion of the paper by heating at over 90°C. The fibres are made from an amino-formaldehyde resin that has been modified by the incorporation of certain inorganic oxyacid, e.g. sulphite, radicals. However the inorganic oxyacid radicals incorporated into the resin reduce the degree of cure of the fibres and so the procedure of FR-A-2373617 suffers from the same disadvantages as the procedures of the aforementioned EP-A-14026 and US-A-4172057.

It has been proposed in GB-A-1574344 to make paper from a mixture of cellulose pulp and urea-formaldehyde (UF) resin fragments, particularly fragments of a UF foam, that have been partially cured by acidification at a temperature below 60°C. After forming the cellulose pulp/UF fragments mixture into sheet form, the latter is heated at above 80°C to effect further curing of the UF resin. It is said that this process gives a continuous chemically bonded network in the paper.

Inter-fibre bonded articles made in accordance with the present invention differ from the products of GB-A-1574344 in various respects.

In the process of GB-A-1574344 the use of a cellulose pulp is essential and it is postulated that a chemical bond is formed between the UF fragments and the cellulose: it is indicated that papers made from non-cellulosic fibres and the fragments have insignificant strength. In contrast inter-fibre bonded articles of significant strength can be made in accordance with the present invention using amino-formaldehyde resin fibres alone or in admixture with non-cellulosic fibrous materials.

Furthermore it is indicated in GB-A-1574344 that the incorporation of the UF fragments gives rise to little or no increase in bulk of the paper: the bulk is said to increase by less than 0.1 cm³g-' for each 10% by weight of UF fragments incorporated. In contrast thereto inter-fibre bonded articles containing amino-formaldehyde resin fibres and cellulose fibres exhibit a significant increase in bulk: the bulk increases by at least about 0.15 cm³g-' for each 10% by weight of amino-formaldehyde resin fibres incorporated. The enhancement in bulk generally becomes more pronounced as the degree of beating of the cellulose pulp increases.

In contrast to the process of GB-A-1574344, in the present invention the amino-formaldehyde resin is in the form of fibres that have been hot cured to a high degree before the shaped article is formed therefrom.

Accordingly the present invention provides a process for making a sheet-like article comprising
(i) forming a solution of an amino-formaldehyde resin free of bound inorganic oxyacid radicals and a curing catalyst therefor into fibres,
(ii) curing said fibres by heating them at above 100°C until the degree of cure (as assessed by the procedure hereinbefore described) is above 93%,
(iii) forming an aqueous pulp by dispersing fibrous material in water, said fibrous material containing at least 5% by weight of said cured amino-formaldehyde resin fibres,
(iv) forming a sheet-like article from said pulp, and
(v) promiting inter-fibre bonding by heating said article at a sufficiently high temperature above 80°C, for sufficient time, and in the presence of a sufficient amount of water above 10% by weight of the total weight of fibrous material present, with the application of pressure, before or during said heating, at least sufficient to cause contact between adjacent fibres, so as to cause at least some of the amino-formaldehyde resin fibres to weld to one another and/or to other fibrous material present at at least some of the points where the fibres touch one another.

While applicants do not wish to be bound by the following theory, it is thought that, in the process of the present invention, at least some of the highly cured amino-formaldehyde resin fibres undergo slight hydrolysis at their surfaces thus rendering them somewhat tacky under the prevailing conditions of temperature and moisture. Where such a tackified fibre contacts, e.g. at a point where fibres cross, another fibre (whether or not the other fibre is another tackified amino-formaldehyde resin fibre) fusion or welding at the intersection occurs. As no tackiness of the fibres is however detected in the final product it is thought that dehydration and recondensation of the tackified fibre surfaces occurs as the heating and drying is continued.

The existence of inter-fibre bonding in water-sensitive articles, e.g. paper containing some cellulosic fibres, can also be assessed by measuring the wet strength of the sample: if inter-fibre bonding has occurred the wet strength of the sample will be increased. It is preferred that the wet strength is increased by at least 25% compared with a similar sample in which no inter-fibre bonding exists. The wet strength of a sample in the form of paper may be measured by Tappi Standard Method T456.

It will be appreciated that where a binder is present in the article the wet strength measurement and probing may not be indicative of the presence of inter-fibre bonding but such inter-fibre bonding can be detected by microscopy.

Where the article contains little or no cellulose fibres, there may be little difference between the wet and dry strengths of the article.

In the process of the invention in order to generate inter-fibre bonding, the article is subjected to the action of water at an elevated temperature.

The fibrous material may be formed into the desired sheet form and then wetted and subjected to the elevated temperature or the article may be formed from an aqueous slurry of the fibrous materials and subjected to the elevated temperature as part of the drying process used to remove the water. Thus in the production of paper-like sheet articles, the paper may be made by a conventional wet-laid process and then subjected to inter-fibre bonding conditions in the drying stages of paper manufacture.

The conditions required to generate inter-fibre bonding vary with the degree of cure of the amino-formaldehyde resin fibres. Thus as the degree of cure increases above 93% by weight, the minimum amount of water in the article required to get inter-fibre bonding increases. As the temperature increases the drying time required decreases.

The temperature should be at least 80°C and is preferably in the range 90 to 180°C. The application of pressure before, or preferably during, the heating step promotes inter-fibre bending. The pressure may vary from just sufficient to ensure good contact between adjacent fibres, typically 0.1 to 50 kg cm-² (0,01 to 4,9 MPa) or more depending upon the water content and the drying conditions. As the applied pressure increases, less water is required. While the application of pressure greater than that, that is just sufficient to ensure good contact between adjacent fibres is not always necessary, its application enables inter-fibre bonding to be obtained in some borderline cases where, in the absence of applied pressure, no inter-fibre bonding is achieved.

The time required may vary from about 30 seconds to 10 minutes or more: it will be appreciated that longer times than the minimum required to achieve inter-fibre bonding may be employed.

The minimum water content required to achieve inter-fibre bonding varies from about 10% by weight of the fibrous material (at low degrees of cure, high temperature and pressure) to over 300% (at low pressures and temperature and high degree of cure). Again it will be appreciated that more water than the minimum required to achieve inter-fibre bonding may be employed. Preferably at least 200% by weight of water is used, based on the dry weight of the fibrous material.

Simple experimentation will enable conditions where inter-fibre bonding results to be determined.

The amino-formaldehyde resin used to make the amino-formaldehyde resin fibres is a condensate of an amino compound, preferably a polyamine such as urea or melamine, with formaldehyde. The amino compound is preferably urea, alone or in admixture with up to 5% by weight of melamine. The molar ratio of formaldehyde to amino groups is preferably between 0.6:1 and 1.5:1 particularly between 0.7:1 and 1.3:1.

The amino-formaldehyde resin fibres may be made by any suitable fibre forming technique such as wet or dry spinning and are preferably formed by a centrifugal spinning process, for example as described in US Patent Specification 4178336, which gives, as is preferred, substantially straight and unbranched fibres.

The amino-formaldehyde resin fibres preferably have an average length, weighted by length, of between 1 and 10 mm, particularly between 2 and 6 mm. Preferably substantially all the amino-formaldehyde resin fibres have a length within the range 1 to 10 mm.

The amino-formaldehyde resin fibres preferably have an average diameter between 1 and 20 pm, particularly between 2 and 15 pm, and most particularly between 3 and 10 ₁1m. Preferably substantially all the amino-formaldehyde resin fibres have a diameter between 1 and 30 pm. The amino-formaldehyde resin fibres preferably have an average strength of at least 50 Mnm-² (which corresponds approximately to 33 Nmg-¹), particularly at least 100 MNm-² (=67 Nmg-¹).

The amino-formaldehyde fibres should have a degree of cure of at least 93%, preferably 94 to 99% by weight. In the process of the present invention, these degrees of cure are achieved by incorporating a suitable curing catalyst, e.g. ammonium sulphate, ammonium chloride, formic acid, dihydrogen ammonium phosphate, or phosphoric, sulphuric, sulphamic, or hydrochloric acids into the resin prior to spinning into fibres and then heating the fibres after spinning at above 100°C, particularly above 120°C for e.g. up to 3 hours: in general the higher the curing temperature, the shorter the time required. Thus while 3 hours at 120°C may give a degree of cure of about 94% by weight, only 5 minutes may be required at 180°C to give a degree of cure of about 97%.

The sheet-like article may be made from the amino-formaldehyde resin fibres as the sole fibrous constituent or may be made from the amino-formaldehyde resin fibres in admixture with other fibrous materials, which may be cellulosic or non-cellulosic. The amino-formaldehyde resin fibres should constitute at least 5% by weight of the total fibrous material in the article.

Particularly useful sheet materials, e.g. paper and board, may be made from blends of amino-formaldehyde resin fibres and cellulose fibres containing 5 to 100%, preferably 10 to 50%, by weight of amino-formaldehyde resin fibres. Cellulose fibres that may be used include the lignin-free fibres such as cotton linters or chemical wood pulp e.g. paper making pulp made from the raw cellulose by treatment by chemical means such as the well known sulphate or sulphite processes, or lignin-containing fibres such as mechanical, semi-chemical, or thermomechanical wood pulp. Mixtures of lignin-containing and lignin-free cellulose fibres, e.g. mixtures of mechanical and chemical pulps, may be used.

The cellulose fibres may be lightly beaten or well beaten, depending on the intended use of the article.

The invention is of particlar merit in the production of sheet like products such as paper and board from fibrous materials comprising amino-formaldehyde resin fibres alone or in admixture with up to 90% by weight, based on the total weight of fibrous material, of cellulose fibres. Such products have improved mechanical properties compared to those in which there is no inter-fibre bonding and, in particular, have superior wet strengths. Thus inter-fibre bonded amino-aldehyde resin fibre containing papers have superior wet strengths to the 100% cellulose papers which have not been otherwise treated to promote wet strength, e.g. by the inclusion of a wet strength resin binder.

As mentioned hereinbefore, in contrast to the papers described in GB-A-1574344, the use of the amino-resin fibres in admixture with cellulose fibres gives a significant increase in bulk. An increase in bulk is generally desirable as it enables less raw materials to be used, with consequent economic advantages, to obtain a paper of given volume. While the bulk of an all-cellulose paper can be increased by reducing the degree of beating of the cellulose, this results in a reduction in paper strength. The incorporation of the amino-formaldehyde resin fibres enables an increase in bulk to be achieved without such a large decrease in paper strength.

As mentioned hereinbefore, the inter-fibre bonded papers of the present invention have improved wet strength compared to papers in which there is no inter-fibre bonding: this renders paper made in accordance with the invention particularly suited to applications such as filter papers. Increased bulk is desirable in such applications as the porosity increases with an increase in bulk.

Articles made in accordance with the present invention from a mixture of amino-formaldehyde resin fibres and cellulose fibres, i.e. cellulose pulp, having a bulk of at least where x is the percentage by weight of amino-formaldehyde resin fibre in the fibrous mixture, and A is the bulk of an article made under similar conditions from the cellulose fibre alone. The increase in bulk given by the incorporation of the amino-formaldehyde resin fibres becomes greater as the degree of beating of the cellulose fibre increases: thus where the cellulose fibre is lightly beaten, so as to give a paper of high bulk, the increase in bulk may be little more than about but with a more highly beaten cellulose pulp, particularly one giving a paper of bulk below about 2 cm³g⁻¹ when made wholly from the cellulose fibre, the increase in bulk is generally at least

Articles made in accordance with the present invention from a mixture of cellulose fibres and amino-formaldehyde resin fibres are preferably made from fibre mixtures containing 5 to 95, particularly 10 to 50, % by weight of amino-formaldehyde resin fibres and, correspondingly, 95 to 5, particularly 90 to 50%, by weight of cellulose fibres.

Articles may also be made in accordance with the present invention from fibrous material containing only amino-formaldehyde resin fibres or amino-formaldehyde resin fibres in admixture with non-cellulosic fibres. These mixtures may, if desired, also contain cellulosic fibres. The non-cellulosic fibres may be synthetic organic fibres such as polyester, e.g. polyethylene terephthalate, fibres; polyolefin, e.g. polypropylene, fibres; or polyamide fibres; or inorganic fibres such as glass or asbestos fibres.

Where non-cellulosic fibres, or a mixture of cellulosic and non-cellulosic fibres are employed, the fibrous material contains at least 5% by weight of amino-formaldehyde resin fibres and, correspondingly, up to 95% by weight of the non-cellulosic fibres or mixture of cellulosic and non-cellulosic fibres. The amount of non-cellulosic fibres is preferably at least 10% by weight of the total weight of fibres in the article. The fibrous material, other than the amino-formaldehyde resin fibres, preferably comprises 10 to 100% by weight of non-cellulosic fibres and, correspondingly, 90 to 0% by weight of cellulosic fibres.

Paper or other sheet like products made in accordance with the present invention from amino-formaldehyde resin fibres alone or from mixtures containing non-cellulosic fibres, have a significant strength whether or not they also contain cellulose fibres. Thus they may have a burst index (bursting pressure measured according to the TAPPI standard procedure divided by the weight per unit area) of at least 0.2 kPa m2g-1..

Where the article contains cellulose fibres in addition to the non-cellulosic fibres, the amino-formaldehyde resin fibres may also be welded to the cellulosic fibres.

Particularly preferred fibre compositions comprise 10 to 90, especially 20 to 60, % by weight of amino-formaldehyde resin fibres, 10 to 90, especially 20 to 50, % by weight of non-cellulosic fibres, and 0 to 75, especially 10 to 50, % by weight of cellulosic fibres.

The invention is illustrated by the following examples in which all percentages are expressed by weight.

### Example 1

A commercially available aqueous urea/formaldehyde resin having a U:F molar ratio of 1:2 of solids content 67% was diluted with water to a viscosity of 30 poise (3 Pa - s). 10%, based on the solids, of an aqueous solution containing 1.6% poly(ethylene oxide) and 6.7% ammonium sulphate was mixed continuously with the resin solution as it was fed to a spinning cup of a centrifugal spinning apparatus. The resin was spun by the process described in US Patent Specification 4178336 using a spinning cup of 12.7 cm diameter having 24 rectangular holes and rotating at 7000 rpm.

Air at 180°C was blown into the spinning chamber to dry the fibres, to transport them from the spinning cup and to effect some curing. The resin was spun at a rate of 100 g min-'. The fibres were continuously removed from the spinning apparatus and their cure was continued by heating in air at 150°C for 40 minutes.

The resultant fibres, which had an average diameter of 8.5 pm, had a degree of curing of 94.6%.

The fibres were cut to a nominal length of 3 mm and dispersed in a standard laboratory pulp disintegrator in water (consistency 1.2%) for 17 minutes.

Paper handsheets (100% UF resin fibres) were made by the standard procedure using the British Standard Handsheet former with the replacement of the standard pressing step with pressing in a press heated to 110°C. Prior to pressing water was sprayed on to the handsheets and the moisture content was determined by weighing the handsheets before and after pressing.

After pressing the Burst Index, and Breaking Lengths of the papers were determined.

Burst Index (burst pressure in kPa divided by the substance in gm-²) was determined according to the standard TAPPI procedure. The Breaking Lengths were measured on an Instron tensile tester (table top model) using samples 15 mm wide with a gauge length of 100 mm. The crosshead speed was 0.5 cm/min.

Inter-fibre bonding was assessed microscopically. Its presence is indicated in the following table by a tick.

### Example 2

Example 1 was repeated using resin fibres cured for 120 minutes at 150°C to give a degree of cure of 96.6%.

### Example 3

Example 1 was repeated using resin fibres cured for 170 minutes at 150°C to give a degree of cure of 97.9%.

### Example 4

Example 1 was repeated using resin fibres cured at 150°C for 330 minutes to give a degree of cure of 99.0%.

### Example 5

Example 1 was repeated using resin fibres cured for 30 minutes at 150°C to give a degree of cure of 96.4%. In each case the pressing time was 3 minutes at 110°C.

### Example 6

Example 1 was repeated using fibres cured for 30 minutes at 150°C to give a degree of cure of 95.9%. In this example the moist sheets were pressed at a pressure of about 0.1 kg cm-² for varying times at various temperatures.

The papers of Examples 1 to 6 that exhibited inter-fibre bonding maintained their integrity when immersed in water and gently agitated: those in which there was no inter-fibre bonding did not.

### Example 7

To demonstrate the improvement obtained in the wet strength of papers made from mixtures of urea-formaldehyde resin fibres and cellulose fibres by the present invention, paper handsheets were made from 80% birch sulphate pulp and 20% urea-formaldehyde resin fibres similar to those used in Example 1. Some of the handsheets were wetted and dried under inter-fibre bonding inducing conditions and the wet breaking length was measured.

The results are shown in the following table.

A similar handsheet made wholly from the birch sulphate pulp had wet breaking length of 0.09 km.

### Example 8

Example 7 was repeated but using a 50/50 mixture of the birch sulphate pulp and the urea- formaldehyde resin fibres.

### Example 9

Papers were made on a pilot paper making machine from mixtures of lightly beaten bleached hardwood sulphate cellulose pulp and urea-formaldehyde resin fibres made by the procedure described in Example 1 and having a degree of cure of 94.6%. The paper was dried under light pressure against cylinders heated to about 100°C. The drying time and moisture content were sufficient to give inter-fibre bonding.

Paper was also made and dried under the same conditions from the lightly beaten cellulose pulp alone. The tensile strengths (wet and dry) in the transverse direction of the paper, i.e. at right angles to the machine direction, and the wet burst index was measured and are quoted in the table as a percentage of the corresponding properties of the all-cellulose paper.

It is seen that the bulk increases by over 0.017 cm³g⁻¹ for each percent of urea-formaldehyde fibres incorporated.

### Example 10

Example 1 was repeated using urea-formaldehyde resin fibres of average diameter 9 11m and 94.9% degree of cure, in admixture with glass or polyethylene terephthalate (PET) fibres, and also, in some cases with softwood sulphate cellulose pulp.

The glass fibres had a mean diameter of 20 µm while the PETfibres were 1.5 denier, drawn, uncrimped fibres that had been washed in warm water to remove any spin finish from their surfaces.

The glass, PET, and urea-formaldehyde fibres were cut to provide a length distribution between 1 and 5 mm by passing the fibres twice through a paper shredding machine with the cutters spaced at a nominal 3 mm.

To promote inter-fibre bonding the sheets were couched from the wire of the sheet former, placed on a non-stick plate, weighed, sprayed evenly with a little deionised water, reweighed and then pressed on each side for 30 seconds using a domestic ironing press at 170°C giving an applied pressure of about 0.1 kg cm-². The weight of the dried paper was determined. The solids content of each sheet entering the press was thus determined, and so the moisture content as a percentage of the total fibre content was calculated.

Two sheets were prepared for each variation in the furnish and the Burst Index was measured at four locations on each sheet, and the average Burst Index was determined.

The results are shown in the following table.

All these papers exhibited inter-fibre bonding between the urea-formaldehyde resin fibres and the glass or PET fibres, and with the cellulose fibres where the latter were also present. All the papers retained their integrity when immersed in water.

### Example 11 (Comparative)

In Example 6 of UK Patent Specification 1573115 the production of paper from a mixture of urea-formaldehyde resin fibres and cellulose pulp on a Fourdrinier paper making machine is described. Examination of a sample of the paper produced in that Example revealed no inter-fibre bonding.

### Example 12

Urea-formaldehyde resin fibres made by the procedure described in Example 1 and having a degree of cure of 94% were mixed, in various proportions with a beaten cellulose pulp and made into handsheets by the British Standard method (which involves air drying at room temperature and does not promote inter-fibre bonding).

Similar sheets were also made but inter-fibre bonding induced by drying the sheets under light pressure against a cylinder heated to about 100°C.

In one series of experiments a ground wood, i.e. mechanical, cellulose pulp was used, which in another series a Kraft, i.e. chemical, pulp was employed. The burst indexes were measured.

It is seen that inter-fibre bonding gives a significant enhancement in the burst index.

## Claims

1. A process for making a sheet-like article comprising
(i) forming a solution of an amino-formaldehyde resin free of bound inorganic oxyacid radicals and a curing agent therefor into fibres,
(ii) curing said fibres by heating them at above 100°C until their degree of cure is at least 93%, as assessed by digesting an accurately weighed sample of about 5 g of the dry fibre in 200 ml of water for 2 hours at 50°C, recovering the undissolved fibre by filtration, drying the recovered fibre at 100°C in air for 2 hours, and expressing the weight of the dry recovered fibre as a percentage of the weight of said sample,
(iii) forming an aqueous pulp by dispersing fibrous material in water, said fibrous material containing at least 5% by weight of said cured amino-formaldehyde resin fibres,
(iv) forming a sheet-like article from said pulp, and
(v) promoting inter-fibre bonding by heating said article at a sufficiently high temperature above 80°C, for sufficient time, and in the presence of a sufficient amount of water above 10% by weight of the total weight of fibrous material present, with the application of pressure, before or during said heating, at least sufficient to cause contact between adjacent fibres, so as to cause at least some of the amino-formaldehyde resin fibres to weld to one another and/or to other fibrous material present at at least some of the points where the fibres touch one another.

2. A process according to claim 1 wherein said inter-fibre bonding is promoted by heating said article at a temperature within the range 90 to 180°C.

3. A process according to claim 1 or claim 2 wherein the inter-fibre bonding is promoted by heating said article in the presence of at least 200% by weight of water, based on the total weight of said fibrous material.

4. A process according to any one of claims 1 to 3 wherein inter-fibre bonding is promoted by subjecting the article to the temperature above 80°C during the drying of the water from the pulp.

5. A process according to any one of claims 1 to 4 wherein the amino-formaldehyde resin fibres have a degree of cure between 94 and 99%.

6. A process according to any one of claims 1 to 5 wherein the pulp contains a mixture of 10 to 50% by weight of amino-formaldehyde resin fibres and correspondingly 90 to 50% by weight of cellulose fibres.

7. A process according to any one of claims 1 to 6 wherein the fibrous material of the pulp comprises 5 to 100% by weight of said amino-formaldehyde resin fibres and correspondingly 0 to 95% by weight of a fibrous material consisting of 10 to 100% by weight of non-cellulosic fibres and correspondingly 0 to 90% by weight of cellulosic fibres.

8. A process according to claim 7 wherein the fibrous material of the pulp comprises 20 to 60% by weight of amino-formaldehyde resin fibres, 20 to 50% by weight of non-cellulosic fibres and 10 to 50% of cellulose fibres.

## Patentansprüche

1. Verfahren zur Herstellung eines blattartigen Gegenstandes, bei dem
(i) aus einer Lösung eines Amino-Formaldehydharzes ohne gebundene anorganische Sauerstoffsäurereste und eines Härtungsmittels dafür Fasern gebildet werden,
(ii) die Fasern ausgehärtet werden, indem sie auf mehr als 100°C erhitzt werden, bis ihr Aushärtungsgrad mindestens 93% beträgt, wobei der Aushärtungsgrad dadurch bestimmt wird, daß eine genau gewogene Probe von etwa 5 g der trockenen Fasern 2 h lang bei 50°C in 200 ml Wasser digeriert wird, die nicht gelösten Fasern durch Filtrieren zurückgewonnen werden, die zurückgewonnenen Fasern 2 h lang bei 100°C an der Luft getrocknet werden und das Gewicht der trockenen, zurückgewonnenen Faser als prozentualer Anteil des Gewichts der Probe ausgedrückt wird,
(iii) durch Dispergieren von Fasermaterial in Wasser ein wäßriger Brei gebildet wird, wobei das Fasermaterial mindestens 5 Gew.-% der ausgehärten Amino-Formaldehydharz-Fasern enthält, (iv) aus dem Brei ein blattartiger Gegenstand geformt wird und
(v) eine Zwischenfaserbindung gefördert wird, indem der Gegenstand für eine ausreichende Zeit auf eine ausreichend hohe Temperatur oberhalb von 80°C und in Gegenwart einer ausreichenden Wassermenge, die mehr als 10 Gew.-% des Gesamtgewichts des vorhandenen Fasermaterials beträgt, erhitzt wird, wobei vor dem Erhitzen oder während des Erhitzens ein Druck ausgeübt wird, der mindestens ausreicht, um eine Berührung zwischen benachbarten Fasern zu verursachen, um zu veranlassen, daß mindestens einige der Amino-Formaldehydharz-Fasern miteinander und/oder mit anderem vorhandenem Fasermaterial an mindestens einigen der Stellen bzw. Punkte, wo die Fasern einander berühren, eng verbunden bzw. verschmolzen werden.

2. Verfahren nach Anspruch 1, bei dem die Zwischenfaserbindung dadurch gefördert wird, daß der Gegenstand auf eine Temperatur in dem Bereich von 90 bis 180°C erhitzt wird.

3. Verfahren nach Anspruch 1 oder 2, bei dem die Zwischenfaserbindung dadurch gefördert wird, daß der Gegenstand in Gegenwart von mindestens 200 Gew.-% Wasser, auf das Gesamtgewicht des Fasermaterials bezogen, erhitzt wird.

4. Verfahren nach einem der Ansprüche 1 bis 3, bei dem die Zwischenfaserbindung dadurch gefördert wird, daß der Gegenstand der oberhalb von 80°C liegenden Temperatur ausgesetzt wird, während zur Entfernung des Wassers aus dem Brei getrocknet wird.

5. Verfahren nach einem der Ansprüche 1 bis 4, bei dem die Amino-Formaldehydharz-Fasern einen Aushärtungsgrad zwischen 94 und 99% haben.

6. Verfahren nach einem der Ansprüche 1 bis 5, bei dem der Brei eine Mischung von 10 bis 50 Gew.-% Amino-Formaldehydharz-Fasern und entsprechend 90 bis 50 Gew.-% Cellulosefasern enthält.

7. Verfahren nach einem der Ansprüche 1 bis 6, bei dem das Fasermaterial des Breis 5 bis 100 Gew.-% der Amino-Formaldehydharz-Fasern und entsprechend 0 bis 95 Gew.-% eines Fasermaterials, das aus 10 bis 100 Gew.-% Nicht-Cellulosefasern und entsprechend 0 bis 90 Gew.-% Cellulosefasern besteht, enthält.

8. Verfahren nach Anspruch 7, bei dem das Fasermaterial des Breis 20 bis 60 Gew.-% Amino-Formaldehydharz-Fasern, 20 bis 50 Gew.-% Nicht-Cellulosefasern und 10 bis 50 Gew.-% Cellulosefasern enthält.

## Revendications

1. Procédé de fabrication d'un article en feuille caractérisé en ce qu'il comprend:
(i) la formation d'une solution d'une résineamino-formaldéhyde dépourvue de radicaux oxyacides inorganiques et d'un agent pour le durcissement de celle-ci en fibres;
(ii) le durcissement de ces fibres par chauffage au delà de 100°C jusqu'à obtention d'un degré de durcissement d'au moins 93%, tel qu'il est établi par la digestion d'un échantillon pesé avec précision d'environ 5 g de fibres sèches dans 200 ml d'eau pendant 2 heures à 50°C, la récupération des fibres non-dissoutes par filtration, le séchage des fibres récupérées à 100°C dans de l'air pendant 2 heures et l'expression du poids des fibres sèches récupérées en pourcentage du poids de l'échantillon; (iii) la formation d'une pâte aqueuse par dispersion du matériau fibreux dans de l'eau, ce matériau fibreux contenant au moins 5% en poids de ces fibres de résine amino-formaldéhyde durcies;
(iv) la formation d'un article en feuille à partir de cette pâte; et
(v) l'initiation d'une liaison inter-fibres par chauffage de l'article à une température suffisamment au-dessus de 80°C pendant une durée suffisante et en présence d'une quantité d'eau suffisante, supérieure à 10% en poids du poids total du matériau fibreux présent, avec application d'une pression avant ou pendant ce chauffage, au moins suffisante pour provoquer un contact entre des fibres adjacentes de façon à provoquer la soudure d'au moins certaines des fibres de résine amino-formaldéhyde les unes avec les autres et/ou un autre matériau fibreux présent, au moins en certains des points où ces fibres se touchent.

2. Procédé suivant la revendication 1, caractérisé en ce que l'on provoque la liaison inter-fibres en chauffant cet article à une température dans la gamme de 90 à 180°C.

3. Procédé suivant l'une quelconque des revendications 1 ou 2, caractérisé en ce qu'on provoque la liaison inter-fibres en chauffant l'article en présence d'au moins 200% en poids d'eau, par rapport au poids total du matériau fibreux.

4. Procédé suivant l'une quelconque des revendications 1 à 3, caractérisé en ce que l'on provoque la liaison inter-fibres en soumettant l'article à une température supérieure à 80°C pendant le séchage éliminant l'eau de la pulpe.

5. Procédé suivant l'une quelconque des revendications 1 à 4, caractérisé en ce que les fibres de résine amino-formaldéhyde présentent un degré de durcissement entre 94 et 99%.

6. Procédé suivant l'une quelconque des revendications 1 à 5, caractérisé en ce que la pulp comprend un mélange de 10 à 50% en poids de fibres de résine amino-formaldéhyde et de façon correspondante, de 90 à 50% en poids de fibres de cellulose.

7. Procédé suivant l'une quelconque des revendications 1 à 6, caractérisé en ce que le matériau fibreux de la pulpe comprend 5 à 100% en poids de fibres de résine amino-formaldéhyde et de façon correspondate, 0 à 95% en poids d'un matériau fibreux consistant en 10 à 100% en poids de fibres non-cellulosiques et de façon correspondante, en 0 à 90% en poids de fibres cellulosiques.

8. Procédé suivant la revendication 7, caractérisé en ce que le matériau fibreux de la pulpe comprend 20 à 60% en poids de fibres de résine amino-formaldéhyde, 20 à 50% en poids de fibres non-cellulosiques et 10 à 50% en poids de fibres cellulosiques.
